

106-79

CROSS REFERENCE

EXAMINER

3

M. L. COSSITT.

MANIFOLDING MEDIUM.

APPLICATION FILED JULY 15, 1919.

1,353,149.

Patented Sept. 21, 1920.

Fig. 1 -



Fig. 2 -



Fig. 3 -

2. Impression giving material  
1. Fabric  
3. Non-impression coating.

WITNESS

Wm G. Drew

INVENTOR

Malcolm L. Cossitt  
BY  
Booth & Booth

ATTORNEYS

X R

## UNITED STATES PATENT OFFICE.

MALCOLM L. COSSITT, OF OAKLAND, CALIFORNIA, ASSIGNOR TO MANIFOLD IMPRESSIONS CORPORATION, OF CARSON CITY, NEVADA, A CORPORATION OF NEVADA.

## MANIFOLDING MEDIUM.

1,353,149.

Specification of Letters Patent. Patented Sept. 21, 1920.

Application filed July 15, 1919. Serial No. 311,060. 117-36

*To all whom it may concern:*

Be it known that I, MALCOLM L. COSSITT, a citizen of the United States, residing at Oakland, in the county of Alameda and 5 State of California, have invented certain new and useful Improvements in Manifolding Mediums, of which the following is a specification.

My invention relates to the manifolding 10 art by which duplicates of writing, typing, printing, drawing, and other inscriptions are made by the transference under pressure of ink, carbon, graphite or other like substances, from a carrier to a surface, to 15 make on the latter visible impressions.

This art is best exemplified by the use, as 20 a manifolding medium, of that article of manufacture known as carbon-paper, and it is to this general class of manifolding media that my invention relates.

The object of my invention is to provide 25 a manifolding-medium as a new article of manufacture, which, while possessing, in common with carbon-paper, the property 30 of transferring an impression to the obverse surface of an underlying sheet and preventing an impression on the reverse surface of an overlying sheet, has the additional advantage, due to its novel preparation, of being adapted for uses for which ordinary 35 carbon paper is unsuited. Though many such uses might be named, it is sufficient to give, as an example, that use which, at present, I deem the most important, namely, 40 that of a manifolding ink-ribbon for type-writing machines of all kinds including calculating machines and all others, using inking ribbons the impressions from which are due to the impact of key-operated type-carrying bars or arms.

In the use of my medium, I am enabled 45 to manifold articles on the machine, without the use of carbon-paper, the manifolding being done on ordinary single sheets of paper inserted in the machine in the usual manner, with my manifolding ribbon or ribbons lying between them.

Though I do not confine myself to this 50 application and use of my invention, I shall for the sake of example, both describe and illustrate my manifolding medium in the form of a ribbon.

Preliminarily, I will state briefly that my 55 invention consists generally in a manifolding medium, as a new article of manufac-

ture, comprising a foundation one surface of which is provided with a suitable impression element, and the opposite surface of which has applied thereto a non-impression element; and it also consists specifically 60 in such article of manufacture, when the non-impression element is in the form of a coating having a gelatin base.

In the accompanying drawing,

Figure 1 is a short-section of a ribbon-like manifolding-medium made in accordance with my invention, showing the obverse or impression element face thereof, which element is omitted in part, to show the foundation.

Fig. 2 is a similar view showing the reverse or non-impression element face.

Fig. 3 is a cross-section of the same.

1 is the foundation of my article. This, in the present example of the invention, is 75 a suitable fabric, from which ink-ribbons are commonly made.

One face of the foundation, which I may consider the obverse face has a coating 2 of transferable-impression material, say, for 80 example ink. The ink may or may not permeate the foundation according to the nature of the latter. In the case of a fabric ribbon the ink would more or less be absorbed.

The other or reverse face of the foundation has applied to it a coating 3 of a non-impression material, say, for example, a gelatin solution, which is not only a non-impression element, but is also non-absorptive of the ink, which in the case of a fabric foundation is essential.

In these drawings, I have necessarily exaggerated the coatings 2 and 3 and the thickness of the foundation 1, and have endeavored by the difference in the shading of the coatings to distinguish their natures.

In the generic aspect of my invention, the foundation 1 may be of any material, according to the use to which the article is to 100 be put.

Also the impression element 2 may be of any kind of material capable of transfer under pressure or impact.

Likewise, the non-impression element 3 105 may be of any material or substance having the property of non-marking under pressure or impact, and when the foundation and impression element are such that the former absorbs the latter, the non-impression ele- 110

ment 3 must be non-absorptive of the impression element.

The non-impression element may be intimately associated with the foundation to form a part of the article in various ways, as for example by the use of a liquid or semi-liquid composition adhering as a true coating, or by the use of a more solid material glued or otherwise caused to adhere to the foundation.

In the preferred and specific manufacture of my manifolding-medium, namely as an ink-ribbon the foundation of fabric has its impression or obverse surface provided or formed in any known way, as for example, its treatment with ink, and it has its non-impression or reverse surface, coated with a composition of matter having a gelatin base, said composition being in its simplest form an aqueous solution of gelatin, but in its more complete form, with the addition of a silicate of potash or soda commonly known as water-glass.

As an example of the preparation of the reverse face of the foundation with an aqueous solution of gelatin, I give 30 grains of gelatin to  $\frac{1}{2}$  ounce of water, forming a soft spongy mass. These ingredients are steamed or cooked at about 110 degrees F. until the gelatin is well dissolved, and after the solution has cooled to about 80 degrees F, it is applied to the foundation.

In case a silicate be added, I give as an

example, 30 grains of gelatin,  $\frac{1}{4}$  oz. of water and  $\frac{1}{2}$  oz. of alkali silicate. This composition is prepared and applied as above stated.

These, as stated, are mere examples, and I am not to be understood as confining myself to these proportions, nor to the details of preparation.

The gelatin coating is cleanly and impervious to ink, so that it will not soil the back of the overlying sheet, nor absorb the ink from the usually saturated foundation. It will not therefore, make an impression on the back of the overlying sheet. It is moreover, flexible, and tough, which properties are enhanced, when a silicate is used in the composition, the effect of which renders it more flexible and less liable to crack.

I claim:

As a new article of manufacture a manifolding medium comprising a foundation having on one side means for transferring visible impressions under pressure, and having on its other side a coating consisting of an aqueous solution of gelatin and an alkali silicate.

In testimony whereof I have signed my name to this specification in the presence of two subscribing witnesses.

MALCOLM L. COSSITT.

Witnesses:

Wm. F. BOOTH,  
D. B. RICHARDS.